

# UNITED STATES PATENT OFFICE.

JOHN ALLEN HEANY, OF YORK, PENNSYLVANIA.

## MANUFACTURE OF LUMINANT FOR ELECTRIC LAMPS.

No. 842,546.

Specification of Letters Patent.

Patented Jan. 29, 1907.

Original application filed December 29, 1904, Serial No. 238,769. Divided and this application filed November 27, 1906.  
Serial No. 345,405.

*To all whom it may concern:*

Be it known that I, JOHN ALLEN HEANY, a citizen of the United States, residing at York, in the county of York and State of Pennsylvania, have invented certain new and useful Improvements in the Manufacture of Luminants for Electric Lamps.

This invention relates to the manufacture of luminants for electric lamps made of very pure refractory metals, such as tungsten, titanium, zirconium, &c., or alloys of two or more of such metals, or of pure chromium, molybdenum, thorium, manganese, or alloys of such metals.

My luminants have properties heretofore unattainable, such as being ductile and capable of standing a much higher temperature than any form of carbon or the carbids of such metals, and are more efficient than any hitherto known metallic filaments. They can withstand a much higher temperature and also convert the heat into light waves, and thereby have the properties of selective radiation. I utilize these metals, or osmium, cerium, niobium, tantalum and vanadium, or boron and silicon, either singly or mixed in a powdered form, as some of these powdered metals can be obtained by known processes, more or less pure, or I can employ the pure oxids, hydrides, nitrides, or metals in a very fine powder or in a colloidal state of the oxid or colloidal suspension of the pure metal, and with the dry powder use a lubricant or binder, such as water or paraffin, to form or shape them. They are then baked in an oven to drive out the paraffin or water, and in case the oxid is used the filament is reduced in pure hydrogen by external heat to the metal. The preliminary baking does not oxidize the metal, but merely strengthens it, and during this operation the binder is dissipated, leaving the filament formed of a refractory substance, strong, durable, and of good conductivity. The body is now heated by an electric current in a vacuum to drive out the hydrogen and to sinter or alloy the particles. If the filament is too large or rough, it may be rolled or drawn to the desired shape.

This application is a division of my previous application for patent, filed December 29, 1904, Serial No. 238,769, and is directed particularly to a pure titanium filament and the method of producing it.

As an illustration of a suitable process, 55 titanium nitrides are produced by known processes—such, for instance, as the titanium dinitrid ( $Ti N_2$ ) may be produced by heating the pure titanium dioxid in pure ammonia-gas, although other titanium nitrides may be employed. The titanium nitrid is mixed with a very small percentage of water or paraffin and heated, as above described, to eliminate the water or paraffin, and the filament is then treated by an electric current in a vacuum to a sufficient temperature to decompose the nitrid, and a dense homogeneous pure titanium filament results, or the pure titanium metal, in a very fine powder, is squirted into shape by means of a suitable lubricant, such as water or paraffin, heated gently to drive out all traces of the lubricant, and then sintered in a vacuum into a dense shiny pure titanium filament, or, if desired, titanium dioxid is converted 65 into the colloidal state and formed into shape, dried by gentle heat, and heated in pure hydrogen to reduce the filament into the metal, although in this last-named operation it is quite probable that some or nearly all of 70 the titanium dioxid is merely reduced to the suboxid ( $TiO$ ); but as this substance is a good conductor of electricity it is admirably suited for further treatment; or the titanium metal is converted into the colloidal state and 75 formed into filaments, when in the desired consistency gently heated, and in both these last-described cases the filament is traversed by a suitable electric current in a vacuum to 80 sinter and shrink the filament into a dense 85 shiny homogeneous metallic filament. 90

The luminant bodies are to be used in a vacuum or neutral gas to prevent any possible oxidization of the metal and give a greater light for the same expenditure of energy or 95 the same light at a much less expenditure of energy than any form of electric luminant hitherto known. This wonderful, and hitherto unknown efficiency may be attributed not only to the high temperature coefficient 100 and the high temperature which the filament can withstand, but also to the shiny metallic surface of the luminant, which radiates the light-rays in a remarkable manner.

Should there be the slightest trace of carbon or of some easily-fusible metal like platinum present in the luminant body, its efficiency will be so reduced as to render the

body almost useless. A trace of carbon may permeate the filament of the lamp during the exhausting operation if care is not taken to prevent the vaporized oil of the pump from entering the bulb of the lamp and combining with the titanium filament.

Having thus described the nature and object of my invention, what I claim as new, and desire to secure by Letters Patent, is—

- 10 1. A filament for incandescent lamps consisting exclusively of metallic titanium in a dense, shiny coherent state and homogeneous throughout.
- 15 2. A filament for electric incandescent lights consisting throughout of substantially pure metallic titanium of high fusing-point and electrically conductive, which is stable at an efficiency at which a carbon filament, or a titanium carbide filament, will rapidly disintegrate, the light-emitting properties of the filament being due to the homogeneous metallic nature of the titanium.
- 20 3. The process of forming a dense, homogeneous titanium filament for electric incandescent lamps which consists in producing a filament which consists exclusively of a titanium compound in the desired shape and then dissociating said titanium compound in an inert environment thereby eliminating the

substance which the titanium has combined with and shrinking the remaining pure metal into a dense, homogeneous shiny filament.

4. The process of forming a dense homogeneous titanium filament for electric incandescent lamps which consists in producing a filament which consists exclusively of a conducting titanium compound in the desired shape, and then dissociating said titanium compound by passing therethrough an electric current in a vacuum thereby eliminating the substance with which the titanium was combined with and by means of said electric current shrinking and sintering the remaining pure metal into a dense homogeneous shiny filament.

5. The process of forming a dense homogeneous titanium filament for electric incandescent lamps which consists in producing a filament which consists exclusively of titanium nitride in the desired shape and then dissociating said nitride in an inert environment thereby eliminating the nitrogen of the nitride and shrinking the remaining pure metal into a dense homogeneous shiny filament.

JOHN ALLEN HEANY.

Witnesses:

HENRY E. EVERDING,  
ROY C. MINGLE.

mt 1

DEPARTMENT OF THE INTERIOR,  
UNITED STATES PATENT OFFICE,  
WASHINGTON, D. C., September 18, 1912.

By a decree of the United States District Court for the Eastern District of Pennsylvania, a copy of which decree is recorded in Liber G 90, page 94, of the Assignment Records of the United States Patent Office, patent No. 842,546, granted to John Allen Heany, was canceled.

EDWARD B. MOORE,  
*Commissioner.*

(*Official Gazette*, September 24, 1912.)